

No. 678,148.

Patented July 9, 1901.

W. A. WARNER.

PROCESS OF PLATING WOOD DOORS.

(No Model.)

(Application filed Sept. 28, 1900.)

Fig. 1.



Fig. 2.



Fig. 3.



Fig. 4.



Fig. 5.



Fig. 6.



Witnesses

*W. V. Devitt*

*R. H. Newman*

Inventor

*William A. Warner*

By  
*Chamberlain & Newman*

Attorneys

# UNITED STATES PATENT OFFICE.

WILLIAM A. WARNER, OF BRIDGEPORT, CONNECTICUT.

## PROCESS OF PLATING WOOD DOORS.

SPECIFICATION forming part of Letters Patent No. 678,148, dated July 9, 1901.

Application filed September 28, 1900. Serial No. 31,375. (No specimens.)

*To all whom it may concern:*

Be it known that I, WILLIAM A. WARNER, a citizen of the United States, and a resident of Bridgeport, in the county of Fairfield and State of Connecticut, have invented certain new and useful Improvements in Processes of Plating Wood Doors, of which the following is a specification.

This invention relates to the process of plating wood doors or like portable articles by means of certain applications, including an electrolytic bath, and has for its object to render the process expeditious, besides producing an improved article.

It is further an object of my invention to provide a process whereby doors or similar articles may be thoroughly plated with a metal deposit, such as copper, brass, or other material, and, further, to produce a door which will be thoroughly inclosed in metal without any visible seams, so as to have the appearance of a solid metal door, yet be cheaper, lighter, and generally more desirable than if it were made of solid metal or covered with sheets, as is now sometimes done. Doors of this class can be extensively used in several places—first, as main-entrance doors to flats or expensive buildings, where grand, massive, and elaborate effects are desired, and internally for fireproof purposes.

The main advantage of doors treated with my invention over the old style of doors is in its lasting quality and the saving of expense each year or two for burning, rubbing down, revarnishing, &c., which is a necessity with the old methods of covering or protecting.

While my invention may be carried into effect by any suitable mechanism which is adapted for the purpose, I have illustrated on an accompanying sheet of drawings three articles which are used in the carrying out of my invention and by means of which the work may be performed expeditiously and practically.

Referring, therefore, to the accompanying sheet of drawings, forming part of this specification, and upon which similar characters of reference denote like or corresponding parts throughout the several views, Figure 1 shows a front and edge view, respectively, of a door trimmed and ready to be completed by my improved process. Fig. 2 is a detailed

front and edge view of the bottom of a door, showing a slight modification of the trimming prior to the electric-plating part of the process. Fig. 3 is a diminutive perspective view of a door with guides secured thereto for supporting the same within the waterproofing and electroplating-tanks which I employ in the carrying out of my process. Fig. 4 is a perspective view, partly broken away, of a tank such as I employ in the carrying out of my process and which is used to submerge the wood article for applying the filler. Fig. 5 is a perspective view of an adjustable table upon which the door is laid for preparing and covering with a conducting material. Fig. 6 is a sectional perspective view of the electroplating-tank in which the door is submerged for the final or electro-plating process.

In the carrying out of my invention upon new doors or other articles to be treated they are first filled with a wood filler of any desired kind—as, for instance, a mixture of linseed-oil and resinous gum—which is designed to waterproof and protect the wood thoroughly and prevent warping. In order to apply this filler, I place it in a tank A, having suitable guides B to retain the door in a true vertical position. Said tank is further fitted with a steam-pipe C for heating the filler and finally with hooks D to engage the supports E on the door F and to retain the same in a submerged position. The doors are placed in the heated filler of this tank and allowed to remain until thoroughly coated and penetrated with the substance, after which they are hoisted, permitted to drain off, and then laid upon the table G for further applications. The door is retained by small shoulders on vertical supports H, carried by the table, one of said supports being secured to an adjustable base I, whereby doors of varying sizes may be accommodated. While contained upon this table in the manner indicated the door is rubbed smooth and coated with varnish, shellac, or other preparatory material and then dried, said operation of rubbing and varnishing being repeated as often as necessary to receive the desired surface. The edges of the door are next trimmed with suitable sheet-metal strips, as indicated in the drawings, wherein J represents a thin metal strip of cor-

responding width to the door attached to the four edges by means of nails, screws, or cement. These metal strips may also be applied to the inner edges K of the panel, if desired, and likewise attached to the front and back face L of the lower edge of the door in such cases where an extra-heavy covering of that part is desired. The material used for this purpose is preferably sheet copper, brass, or bronze, and the strips are obviously shaped to conform and fit to the edges of the door, including the mortises, if desired. After this sheet metal is applied in the places desired the entire door is prepared to receive the electrodeposits, as follows: The face of the strip on the edge of the door is preferably covered with a metallic insulating material, such as wax or asphalt and varnish, after which the entirety is coated with a metal substance, such as thin metallic leaf, metallic bronze-powder, or common varnish or wax with plum-bago. When the coatings applied as above become dry, the door is rinsed and ready to receive the electrodeposit. The electrodeposit or final coating of the door is applied in the tank M, where the door is supported in a somewhat similar manner to that shown in the preceding tank, being supported in a manner to retain the door in a true vertical position, and for this purpose a non-conducting lining N is used within the guides O, together with such other further insulations as may be found necessary. Beside the door and within the tank I provide a supporting-rod P, having attached thereto an electric conducting-wire Q, and to this supporting-rod is attached the metallic plate R, designed to be dissolved and deposited upon the door. The second conducting-wire S, by means of which the complete circuit is formed, is preferably attached to the metal strip upon one edge of the door, and thus it will be seen that when the wires are attached to a suitable dynamo (not shown) the metal is dissolved from the plate and deposited upon the door, where it is finally distributed over its entire surface to any thickness desired, in accordance with the amount of the metal employed and length of the operation. The advantages obtained by covering the edges of the door with a sheet-metal strip are, first, its high conductivity of electric current, making a complete circuit around the door, which acts as a "starter," so to speak, for the deposition of the copper, and, second, the width of the metal strip can be the same as the thickness of the door, thus insuring an even and unbroken surface between the

two. Furthermore, with the strip arranged upon all sides of the door and the face of the same covered with metallic substances a uniform deposit is secured upon the entire face. Were the metal connections made upon the face of the door directly opposite the anodes and without the use of the metal strip, a heavier deposit would be secured at that point and a very light one upon the edges of the door. It is desirable, of course, to have the deposit over the entire door as near uniform as possible; but if there is to be any deviation it should be preferably heavier upon the edges, since there is where the greatest amount of wear comes.

It will be obvious that the details of my invention may be varied without departing from the true essence thereof, and for that reason I do not wish to be limited in any way to the article shown for carrying out the invention or, in fact, to the exact method of filling the wood, since that might be done with a brush, if preferred.

Having thus described my invention, what I claim, and desire to secure by Letters Patent, is—

1. The herein-described process of metal-plating wood doors which consists in first filling the same, then covering the edges with thin metal strips, next covering said door with a thin layer of conducting material, and finally subjecting the whole to an electroplating-bath whereby an electrodeposit is formed over said conducting-layer.

2. The process of plating wood doors or similar articles, which consists first in filling said door, second in applying to the edges thereof thin metal strips, third, insulating the face of said strips, fourth applying a coating of metallic bronze-powder to the face of the door, and finally in electrically depositing a metal coating on the faces of said door.

3. The herein-described process of metal-plating wood doors which consists in first filling the same, next covering the edges with thin metallic strips, third in covering the faces of the door up to the edge of said metal strips with metallic bronze-powder, and finally in electrically depositing a metal coating on said door.

Signed at Bridgeport, in the county of Fairfield and State of Connecticut, this 24th day of September, A. D. 1900.

WILLIAM A. WARNER.

Witnesses:

C. M. NEWMAN,  
W. V. DEVITT.